

April 16, 1968

F. R. THOMANEK

3,377,953

## DETONATOR

Filed July 13, 1966



INVENTOR  
Franz Rudolf Thomanek

by *John and Token*  
ATTORNEYS

1

3,377,953  
DETONATOR

Franz Rudolf Thomaneck, Sandizell 38 1/4, Landkreis  
Schrobenhausen, Upper Bavaria, Germany  
Filed July 13, 1966, Ser. No. 564,871  
Claims priority, application Germany, Aug. 12, 1965,  
B 83,239

7 Claims. (Cl. 102—70)

## ABSTRACT OF THE DISCLOSURE

A detonator is constructed to have a point initiation of the detonation and is arranged to provide for subsequent detonation waves which extend axially symmetrically in the explosive charge. For this purpose a conical tip of a fast acting explosive charge is arranged in a slow acting explosive charge and the means for initiating a detonation is located on a point of the slow acting explosive charge at a location close to the axis of the fast acting explosive charge.

## Summary of the invention

This invention relates, in general, to the construction of an explosive charge and, in particular, to a new and useful explosive charge or detonator having punctiform initiation of the detonation of a high intensity charge for obtaining an axially symmetrical detonation and wherein the explosive charge includes a fast acting explosive embedded in a slower acting explosive.

In order to release in an explosive charge a detonation wave which meets the highest precision standards, it is necessary that the detonation waves start geometrically exactly and that the intensity of the initiation be as high as possible so that the detonation wave can propagate in any direction at full velocity. Only by insuring both criteria will a satisfactory design of detonation wave be possible.

Tests have shown that hollow charges are particularly sensitive to unsymmetrical detonation waves. For this reason, it has been attempted to make the detonation wave as punctiform as possible, for example, by selecting a thin rod-shaped detonator. Therefore, there is a limitation on the diameter of the rod which may be employed and no detonation will be possible with a rod below a certain diameter depending on the properties of the explosive and of the inert tamping (metal case of the detonator). The better the punctiform initiation, the weaker will be the intensity of the detonation wave so that different starting distances in the individual directions will be the effect. The result is therefore an accidentally-formed, that is, an unsymmetrical detonation wave. If the diameter of the detonation rod is increased, the symmetry of the detonation start will improve because the initiation intensity has increased. However, the starting point of the detonation wave will then be equally probable over the entire cross section of the surface contact of the detonator rod. Therefore, because the starting point remains uncertain, it would be impossible to achieve a symmetrical detonation wave.

In accordance with the present invention, there is provided a detonator having punctiform initiation of the detonation of high intensity which includes an explosive charge of a faster detonation velocity explosive imbedded in a charge of a slower acting explosive. Such a construction assures an exact punctiform initiation of the detonation with such a high initiation intensity, that a uniform propagation of the detonation in all directions will occur. This is effected by a detonator which consists of the two explosives of different detonation velocity.

Accordingly it is an object of the invention to provide

2

a detonator having a uniform propagation of detonation in all directions.

A further object of the invention is to provide a detonator having exact punctiform initiation of the detonation with such a high initiation intensity that a uniform propagation of the detonation in all directions will be insured.

A further object of the invention is to provide a detonator which is simple in design, rugged in construction and economical to manufacture.

The various features of novelty which characterize the invention are pointed out with particularity in the claims annexed to and forming a part of this specification. For a better understanding of the invention, its operating advantages and specific objects attained by its use, reference should be had to the accompanying drawings and descriptive matter in which there are illustrated and described preferred embodiments of the invention.

In the drawings:

20 FIG. 1 is a schematic sectional representation of a detonator constructed in accordance with the invention;

FIG. 2 is a view similar to FIG. 1 of another embodiment of the invention; and

25 FIG. 3 is a view similar to FIG. 1 of still another embodiment of the invention.

Referring to the drawings, in particular, the invention embodied therein comprises a detonator which includes a slower explosive 1 of a relatively large size in which is embedded a conical tip 2' of a faster acting explosive 2.

30 The construction, in accordance with the invention, is such that a non-symmetrical detonation is not probable. If an eccentric detonation wave is started, for example, at the tip of the arrow 3, the wave which is propagated designated 4 will strike after a short period of time the tip 2' of the explosive 2. Since the conical tip 2' of the faster-acting explosive 2 is surrounded on all sides by the slower acting explosive 1, the release of the detonation wave in the cone apex takes place with full intensity. The detonation wave shows then at a later point a course or wave path indicated 5. Thus, despite the originally eccentric detonation wave in the explosive 1, an axially symmetrical eccentric detonation wave is released in the cone apex. The following explosive charge proper is therefore initiated axially symmetrically by the symmetrically oriented detonation wave front portion 5a.

35 In the embodiment of the invention indicated in FIG. 1, it is possible to rectify detonation initiations within 3.5 mm. eccentricity as shown by tests.

40 In FIG. 2 another embodiment is indicated in which a slower explosive 7 surrounds a cone apex 8' of a faster acting explosive 8. An additional cone of a faster-acting explosive 9 is arranged above the cone 8 in an apex manner. With this design of detonator as shown in FIG. 2, even greater eccentricities can be rectified so that the problem of a punctiform initiation with high intensity is possible.

45 As an example, the following explosives are used: For the detonator part 7, tetryl pressed with about 2% wax and graphite; for the detonator part 8, for example, a cast explosive of from about 15% TNT and 85% hexogen with a grain size of less than 100  $\mu\text{m}$ . The part 9 may advantageously comprise a highly pressed nitropenta with 2% wax.

50 The detonator according to FIG. 2 operates so that each detonation wave in part 9, no matter where it is released on the surface, is always conducted first to the cone apex of the part 9 and thus also to the apex of the part 8. The detonation waves in part 7 can thus have no harmful effect in any case on the axial symmetrical design of the detonation wave in part 8.

55 The invention described by way of example in respect to an axially symmetrical detonator can be applied to all

other detonators, for example, for releasing a ring-shaped detonation (cylindrical detonation wave).

In the embodiment of FIG. 3, initiation of the detonation in a conical explosive charge of a faster explosive 10 is conducted to the apex of the latter where an annular body 11 of a faster explosive is assembled with intermediate bodies 12 and 13. The intermediate bodies 12 and 13 are made of a slower acting explosive.

In accordance with still a further embodiment of the invention, the individual charges in FIGS. 1 and 2 are joined together, preferably with an adhesive such as a plastic adhesive.

While specific embodiments of the invention have been shown and described in detail to illustrate the application of the inventive principles, it will be understood that the invention may be embodied otherwise without departing from such principles.

What is claimed is:

1. A detonator having punctiform initiation of the detonation of high intensity for obtaining an axially symmetrical detonation, comprising a slow acting explosive charge, and a fast-acting explosive charge having a conical tip imbedded within the slow acting charge, and means for initiating detonation at a point on said slow acting explosive charge at a location close to the axis of said fast acting explosive charge.

2. A detonator, according to claim 1, wherein there are at least two slow acting explosive charges, one each surrounding the respective conical tip portion of each fast-acting explosive charge.

3. A detonator, according to claim 1, including adhesive means bonding said explosive charges together.

4. A detonator, according to claim 1, wherein said fast-acting explosive is a cast explosive of around 15% TNT and 85% hexogen.

5. A detonator having punctiform initiation of a detonation of high intensity, for obtaining an axially symmetrical detonation, comprising a slow acting explosive charge, and a fast-acting explosive charge imbedded within the slow acting charge, said fast-acting explosive charge including a conical tip imbedded in said slow acting charge, and a second fast-acting explosive having a conical tip portion arranged with its apex abutting the apex of said first fast-acting explosive charge, said slow acting explosive charge surrounding the conical tip of said fast-acting and said second fast-acting explosive charges.

10 6. A detonator having punctiform initiation of the detonation of high intensity for obtaining an axially symmetrical detonation, at least two fast-acting explosive charges each having conical tip portions and being arranged with their apexes abutting, and a plurality of slow acting explosive charges surrounding the conical tip portions of said fast-acting explosive charges.

15 7. A detonator, according to claim 6, wherein one of said fast-acting explosives is a cast explosive of around 15% TNT and 85% hexogen and the other is pressed with a nitropenta and 2% wax, and the slow acting explosive is pressed tetryl and 2% wax and graphite.

25

#### References Cited

##### UNITED STATES PATENTS

|           |         |         |       |           |
|-----------|---------|---------|-------|-----------|
| 2,396,978 | 3/1946  | Amthor  | ----- | 102—56    |
| 2,604,042 | 7/1952  | Cook.   |       |           |
| 3,100,445 | 8/1963  | Poulter | ----- | 102—24    |
| 3,285,012 | 11/1966 | Larue   | ----- | 102—101 X |

BENJAMIN A. BORCHELT, Primary Examiner.

V. R. PENDEGRASS, Assistant Examiner.

35